# EUROPEAN PATENT SPECIFICATION

(11) **EP 2 930 260 B1**
(45) Date of publication and mention of the grant of the patent: **16.08.2017**
(21) Application number: 15170904.5
(22) Date of filing: 19.09.2012
(51) Int. Cl.: D04H 1/46, D04H 13/00, D04H 1/425, D04H 1/4258

(54) **FIBROUS ABSORBENT MATERIAL AND METHOD FOR MAKING**
SAUGFÄHIGES FASERMATERIAL UND VERFAHREN ZUR HERSTELLUNG
MATÉRIAU ABSORBANT FIBREUX ET PROCÉDÉ DE FABRICATION

(30) Priority: 20.09.2011 US 201113236799; 20.09.2011 US 201113236788
(43) Date of publication of application: 14.10.2015
(62) Divisional of application: 12184937.6
(73) Proprietor: Johnson & Johnson Consumer Inc., Skillman, NJ 08558 (US)
(72) Inventor: Fung, Paul Y., 14P New York 10025, NY (US)
(74) Representative: Carpmaels & Ransford LLP

(56) References cited:
- EP-A2- 0 525 676
- US-A- 5 928 973
- US-A1- 2009 000 643
- US-A1- 2011 150 558

## Description

### FIELD OF THE INVENTION

The present invention generally relates to a method for making an absorbent material.

### BACKGROUND OF THE INVENTION

Lofty, resilient, non-woven webs, that is nonwoven webs that have a high degree of loft and the tendency to retain such loft, are well known. In addition, it is well known that such lofty, resilient, non-woven webs may be used in disposable sanitary products such as sanitary napkins, pantiliners, tampons, diapers, adult incontinence products, and the like. A perceived benefit of such lofty, resilient, non-woven webs is that such materials may deliver enhanced comfort to a user of such disposable sanitary products since the lofty, resilient, nonwoven webs may tend to conform to, and move with, the user's body during use.

A problem with lofty, resilient, nonwoven webs is that due to the loft of such materials (i.e. their low density) such webs are not particularly absorbent. In addition, such materials may exhibit poor rewet properties. That is, such materials may release or "wet back" fluid when subjected to an external pressure.

In view of the foregoing there is a need for a lofty, resilient, non-woven web that also provides superior fluid handling characteristics.

US 2009/0000643 A1 discloses a cleaning article for moist or wet cleaning comprising a nonwoven, and its use for cleaning human skin or household surfaces or for cleaning surfaces in industrial applications.

US 2011/0150558 A1 discloses a kit comprising a product dispenser for dispensing a personal care composition in combination with an absorbent article.

US 5 928 973 A discloses a non-woven needlepunch fabric consisting essentially of 60% to 90% by weight lyocell fiber having a length of 2.54 cm (one inch) to 15.24 cm (six inches), 10% to 40% by weight polyester fiber having a length of 2.54 cm (one inch) to 15.24 cm (six inches) and 0% to 30% of other textile fibers, wherein said lyocell fiber has a denier in the range of 0.75 to 6 prior to fibrillation, said fabric having been formed by subjecting said fiber to carding, cross-lapping and needle punching to produce a fabric with interlocked fibers.

EP 0 525 676 A2 discloses a facing material suitable for use in diapers and the like which comprises a fibrous top layer for engaging a body fluid, a generally opaque aperture middle layer, and a bottom layer having a capillary structure for drawing body fluid from the fibrous top layer.

### SUMMARY OF THE INVENTION

In view of the foregoing, the present disclosure provides an absorbent material including a fibrous material having a plurality of individual fibers forming a fiber matrix, a plurality of absorbent fibers, wherein the plurality of absorbent fibers are impregnated within the fiber matrix by means of a needlepunch process.

The present disclosure also provides a fibrous material including a plurality of individual fibers forming a fiber matrix, a first plurality of absorbent fibers arranged in a first layer, a second plurality of absorbent fibers arranged in a second layer, wherein the first and second plurality of absorbent fibers are impregnated within the fiber matrix by means of a needlepunch process.

The present invention provides a method for making an absorbent material including the steps of providing a fibrous material including a plurality of individual fibers forming a fiber matrix, depositing a plurality of absorbent fibers on a top surface of the fibrous material, and impregnating the plurality of absorbent fibers into the fiber matrix by means of a needlepunch process wherein each of the plurality of individual fibers has a fiber diameter that is at least 1 µm greater than a fiber diameter of each of the absorbent fibers.

### BRIEF DESCRIPTION OF THE DRAWINGS

Examples of embodiments of the present invention will now be described with reference to the drawings, in which:
Fig. 1 is a sectional schematic view of an absorbent material prepared according to the method of the present invention;
Fig. 2 is a schematic view of an apparatus for making the absorbent material shown in Fig. 1;
Fig. 3 is a schematic view of the encircled portion of the apparatus shown in Fig. 2 depicting a needle employed in the apparatus, a top surface of a substrate, and absorbent fibers arranged on the top surface of the substrate;
Fig. 3a is a detailed view of the encircled portion of the needle shown in Fig. 3;
Fig. 3b-3e depict the manner in which the needle impregnates the absorbent fiber within the substrate;
Fig. 4 is a sectional schematic view of an absorbent material prepared according to the method of the present invention;
Fig. 5 is a sectional schematic view of an absorbent material prepared according to the method of the present invention; and
Fig. 6 is a schematic view of an apparatus for making the absorbent material shown in Fig. 5.

### DETAILED DESCRIPTION OF THE INVENTION

Throughout the present specification, the same or similar reference numbers have been used to identify the same or similar elements of the various embodiments of the present invention described herein.

Reference is made to Fig. 1 which illustrates a sectional schematic view of an absorbent material 10 prepared according to the method of the present invention. As shown in Fig. 1, the absorbent material 10 is formed from a fibrous material 12 including a plurality of individual fibers 14 that form a fiber matrix 16. The absorbent material 10 further includes a plurality of absorbent fibers 18. As shown, the absorbent fibers 18 are impregnated within the fiber matrix 16.

The fibrous material 12 is preferably a fibrous nonwoven material made by a known nonwoven manufacturing technique such as an airlaid process, a card and bind process or a resin and adhesive bond process. Preferably the nonwoven material is a "high loft" nonwoven. Specifically, the nonwoven preferably has a density lower than 0.05 g/cc, and preferably between about 0.01 g/cc and 0.03 g/cc, prior to the impregnation of the nonwoven with the absorbent fibers 18. The individual fibers 14 forming the fibrous nonwoven material may be selected from fibers including synthetic, nonabsorbent fibers that may or may not be wettable, for example hydrophilic fibers, hydrophobic fibers, and combinations thereof. Specific fiber types include, but are not limited to, polyester, nylon, co-polyester, polyethylene, polypropylene, and polylactic acid. Of course the fibrous nonwoven material may be formed from a single nonabsorbent fiber type listed above or alternatively may be formed from a mixture of the fiber types listed above. The surface of nonabsorbent fibers 14 forming the fibrous material 12 may be rendered wettable by treating such fibers with a suitable surface treatment, such a surfactant or like.

Each of the fibers 14 forming the fibrous nonwoven material preferably has a fiber diameter within the range of 11 µm and 100 µm. The fibrous material 12 preferably further includes a binder material, such as a latex binder. The binder material is preferably present in the fibrous material 12 in an amount between about 30% by weight to about 50% by weight.

The absorbent fibers 18 are preferably selected from cellulosic fiber types, such as, but not limited to, hard wood pulp, soft wood pulp, rayon, and cotton. The absorbent material 10 may include a single absorbent fiber type of those listed above or in the alternative may include multiple fiber types of those listed above (i.e. a mixture of absorbent fibers). Each of the absorbent fibers 18 preferably has fiber diameter within the range of 10 µm and 40 µm.

The individual fibers 14 forming the fibrous material 12 and the absorbent fibers 18 are selected such that each of the individual fibers 14 has a fiber diameter that is at least 1 µm greater than a fiber diameter of each of the absorbent fibers 18.

As will be discussed in greater detail below, the absorbent fibers 18 are impregnated within the fiber matrix 16 by means of a needlepunch process according to the present invention. The needlepunch process according to the present invention, described in detail below, allows the absorbent fibers 18 to be impregnated within the fiber matrix 16 without the fibrous material 12 losing its high loft properties. Specifically, the density of fibrous material 12 prior to being impregnated with the absorbent fibers 18 is preferably within the range of 0.01 g/cc and 0.03 g/cc.

The fibrous material 12 preferably has a thickness in the range of about 1.5 mm to about 5 mm prior to impregnation of the fibrous material 12 with the absorbent fibers 18. After impregnation of the fibrous material 12 with the absorbent fibers 18 the absorbent material 10 retains substantially the same thickness as the original fibrous material. Specifically, a percent change between the thickness of the fibrous material 12 prior to the plurality of absorbent fibers 18 being impregnated therein and a thickness of the absorbent material 10 after the absorbent fibers 18 have been impregnated within the fibrous material 12 is preferably less than 50%, more preferably less than 30% and most preferably less than 15%. This relatively small change in thickness reflects that the absorbent material 10 retains the high loft properties of the fibrous material 12 while at the same time delivers superior fluid handling capabilities. The percent change in thickness is calculated as follows: $% ΔT = \left(Ti-Tf\right) / Ti ;$ where
Ti = Initial Thickness of Fibrous Material 12
Tf = Final Thickness of Absorbent Material 10

A method of making the absorbent material 10 will now be described with reference to Fig. 2 which depicts a schematic representation of an apparatus 19 for making the absorbent material 10. As shown in Fig. 2, a web of fibrous material 12 is fed from a supply roll 20 and conveyed in a machine direction by a plurality of rolls 22, 24 and 26. A gravity fed hopper 28, or the like, is utilized to apply a selected amount of absorbent fibers 18 to a top surface 30 of the fibrous material 12. Thereafter, the fibrous material 12 is further conveyed in a machine direction and passed through a conventional needlepunch apparatus 32 of the type known to those of skill in the art. In the method according to the present invention, the needlepunch apparatus 32 functions to impregnate the absorbent fibers 18 within the fibrous material 12 by means of a plurality of needles 34.

As is known to those of skill in the art, a conventional needlepunch apparatus includes a plurality of needles that are normally adapted to mechanically orient and interlock the fibers of a spunbonded or carded web. In the method according to the present invention, the needles 34 of the needlepunch apparatus 32 are used to impregnate absorbent fibers 18 within the fibrous material 12. A needle 34 suitable for use in the method according to the present invention is depicted in Fig. 3 and Fig. 3a. As shown in Fig. 3a, the needle 34 generally includes a blade 36, a barb 38, and a throat section 40. The total barb depth of the barb 38 is indicated by letter "d" in the Fig. 3a.

For purposes of the present invention, it is critical that the barb depth "d" is selected such that a radius of each of the absorbent fibers 18 is smaller than the barb depth "d". The radius of each absorbent fiber 18 is at least 0.5 µm smaller, for example 1 µm smaller than the barb depth. In addition the barb depth "d" should be selected such that each of the individual fibers 14 of the fibrous material 12 has a radius that is larger than the barb depth "d". The radius of each individual fiber 14 of the fibrous material 12 is at least 0.5 µm larger, for example 1 µm larger than the barb depth. If you have a multiple denier fibrous material 12, the diameter of the smallest diameter fiber 14 must be larger than the diameter of each of the absorbent fibers 18.

By selecting barb depth "d" as described above, the plurality of needles 34 in the needlepunch apparatus effectively grasp the absorbent fibers 18 and thus can impregnate such absorbent fibers 18 within the fibrous material 12, as shown in Figs. 3b-3e. On the other hand, the plurality of needles 34 will not grasp the individual fibers 14 of the fibrous material 12 and thus will not destroy the "high loft" properties of the fibrous material 12. In this manner the final absorbent material 10 is provided with superior fluid handling properties while still retaining the high loft properties of the fibrous material 12. Needles particularly useful in the present method are commercially available from the Foster Needle Co., Inc., Manatowoc, Wisconsin, under product designation "The Foster Formed Barb".

Referring again to Fig. 2, after the fibrous 12 has been impregnated with the absorbent fibers 18 the resultant absorbent material 10 is further conveyed in a machine directly by rolls 28 and 30. At this point in the process the absorbent material 10 may be arranged in a rolled form for storage or may be further conveyed for incorporation into disposable sanitary absorbent products such as a sanitary napkin, pantiliner, tampons, diaper, adult incontinence product, or the like.

Alternatively, as shown in Fig. 2, the fibrous material 12 may be further conveyed to a superabsorbent application station 42. The superabsorbent application station 42 comprises a gravity fed hopper 44 structured and arranged to apply a selected amount of superabsorbent polymer material 46 to a top surface 30 of the fibrous material 12. Of course, any suitable means known to those of skill in the art, such as a pressure fed nozzle or the like, may be used to apply the superabsorbent polymer material 46 to the top surface 30 of the fibrous material 12. After the superabsorbent polymer material 46 is applied to the top surface 30 of the fibrous material 12, the fibrous material 12 is conveyed over a vacuum 50 that functions to draw the superabsorbent polymer material 46 into the fiber matrix 16 of the fibrous material 12. The resultant absorbent material 10a, is shown in Fig. 4. As shown, the superabsorbent polymer 46 has been drawn into the fiber matrix 16 of the fibrous material 12 and functions to further enhance the fluid handling capabilities of the absorbent material 10a.

For the purposes of the present invention, the term "superabsorbent polymer" (or "SAP") refers to materials which are capable of absorbing and retaining at least about 10 times their weight in body fluids under a 0.5 psi pressure. The superabsorbent polymer particles of the disclosure may be inorganic or organic crosslinked hydrophilic polymers, such as polyvinyl alcohols, polyethylene oxides, crosslinked starches, guar gum, xanthan gum, and the like. The particles may be in the form of a powder, grains, granules, or fibers. Preferred superabsorbent polymer particles that may be used are crosslinked polyacrylates, such as the product offered by Sumitomo Seika Chemicals Co., Ltd. of Osaka, Japan, under the designation of SA70.

Referring again to Fig. 2, after the absorbent material 10a is conveyed past the vacuum 50 the absorbent material 10a may be further conveyed in a machine direction by roll 51 and arranged in a rolled form for storage or may be further conveyed for incorporation into a disposable sanitary absorbent products such as a sanitary napkin, pantiliner, tampons, diaper, adult incontinence product, or the like.

Reference is made to Fig. 5 which illustrates a sectional schematic view of an absorbent material 10b prepared according to the method of the present invention. As shown, the absorbent material 10b is formed from a fibrous material 12 including a plurality of individual fibers 14 that form a fiber matrix 16. The absorbent material 10b further includes a first plurality of absorbent fibers 18a arranged in a first layer 52 and a second plurality of absorbent fibers 18b arranged in a second layer 54. The absorbent fibers 18a and 18b may comprise the same fibers as those absorbent fibers 18 described above with regard to Fig. 1. The absorbent fibers 18a and 18b may be the same fiber type or may be different fibers types (i.e. a mixture of fibers). In addition, a first absorbent fiber mixture (or individual fiber) may be employed in the first plurality of fibers 18a and different absorbent fiber mixture (or individual fiber) may be employed in the second plurality of fibers 18b.

The individual fibers 14 may be the same as the fibers 14 described above with regard to Fig. 1. In addition the individual fibers 14 may be the same fiber type (i.e. a single fiber type) or different fiber types (i.e. a mixture of fibers).

In Fig. 5, the first layer 52 is arranged in spaced relationship to the second layer 54. The absorbent material 10b may optionally further include superabsorbent polymer material 46 dispersed within the fiber matrix 16 of the fibrous material 12. In Fig. 5, the superabsorbent 46 is arranged in a layer 56 between the first layer 52 and second layer 54 of the absorbent fibers 18a and 18b. Of course the superabsorbent polymer material 46 may be omitted from the absorbent material 10b if desired.

A method of making the absorbent material 10b will now be described with reference to Fig. 6 which depicts a schematic representation of an apparatus 19a for making the absorbent material 10b. As shown in Fig. 6, a web of fibrous material 12 is fed from a supply roll 20 and conveyed in a machine direction by a plurality of rolls 22, 24 and 26. A gravity fed hopper 28, or the like, is utilized to apply a selected amount of absorbent fibers 18a to a top surface 30 of the fibrous material 12. Thereafter, the fibrous material 12 is further conveyed in a machine direction and passed through a needlepunch apparatus 32 for impregnating the absorbent fibers 18a within the fibrous material 12.

Thereafter the fibrous material 12 is further conveyed to a superabsorbent application station 42. The superabsorbent application station 42 comprises a gravity fed hopper 44 structured and arranged to apply a selected amount of superabsorbent polymer material 46 to a top surface 30 of the fibrous material 12. Of course, any suitable means known to those of skill in the art, such as a pressure fed nozzle or the like, may be used to apply the superabsorbent polymer material 46 to the top surface 30 of the fibrous material 12. After the superabsorbent polymer material 46 is applied to the top surface 30 of the fibrous material 12 the fibrous material 12 is conveyed over a vacuum 50 that functions to draw the superabsorbent polymer material 46 into the fiber matrix 16 of the fibrous material 12. Of course, if the inclusion of superabsorbent polymer material 46 is not desired in the absorbent material 10b, the superabsorbent application and vacuum step described may be omitted from the described method.

After the fibrous material 12 is conveyed past the vacuum 50, the fibrous material 12 is conveyed by rolls 51 and 53 to a second gravity fed hopper 28a, or the like, to apply a selected amount of absorbent fibers 18b to a top surface 30 of the fibrous material 12. Thereafter, the fibrous material 12 is further conveyed in a machine direction by rolls 55 and 57 and passed through a second needlepunch apparatus 32a for impregnating the absorbent fibers 18b within the fibrous material 12.

Referring again to Fig. 6, after the absorbent material 10b is conveyed past the needlepunch apparatus 32a the absorbent material 10b is further conveyed in a machine direction by roll 59 and then may be arranged in a rolled form for storage or may be further conveyed for incorporation into a disposable sanitary absorbent products such as a sanitary napkin, pantiliner, tampons, diaper, adult incontinence product, or the like.

### EXAMPLES

Specific examples of the present invention are described below.
Inventive Example #1 - An absorbent material as described above with reference to Figs. 1 and 2 is made as follows. The fibrous material is a fibrous nonwoven made by a card and bind process having a basis weight of 68 gsm, formed from 100% polyester fibers (6 denier), and having a thickness of 3 mm. Given that the density of polyester is 1.38 g/cc, a 6 denier fiber has a nominal diameter of 25 µm (denier = density * 0.0283 r²). The fibrous material includes a latex binder present in the amount of 40% by weight. A fibrous nonwoven material of this type is commercially available from Kem-Wove, Inc., Charlotte, NC under product code SCN09-038. The absorbent fibers comprise 100% viscose rayon having a denier of 4. Rayon has a density of 1.5 g/cc thus the absorbent fibers have a fiber diameter of 19 µm. 150 gsm (g/m²) of the rayon fibers are applied to a top surface of the fibrous nonwoven material and impregnated within the material to a depth of 2.5 mm by means of the needlepunch process described above with reference to Fig. 2. The needles used in the needlepunch process have a barb depth "d" of 12 µm. The final absorbent material has a thickness of 2.7 mm.
Inventive Example #2 - An absorbent material as described above with referenced to Figs. 5 and 6 is made as follows. The fibrous material is a fibrous card and bind nonwoven material having a basis weight of 68 gsm, formed from 100% polyester fibers (6 denier), and having a thickness of 3 mm. Given that the density of polyester is 1.38 g/cc, a 6 denier fiber has a nominal diameter of 25 µm (denier = density * 0.0283 r²). The fibrous material includes a latex binder present in the amount of 40% by weight. A fibrous nonwoven material of this type is commercially available from Kem-Wove, Inc., Charlotte, NC under product code SCN09-038. The first plurality of absorbent fibers comprises 100% viscose rayon having a denier of 4. Rayon has a density of 1.5 g/cc thus the absorbent fibers have a fiber diameter of 19 µm. 75 gsm of the rayon fibers are applied to a top surface of the fibrous nonwoven material and impregnated within the material to a depth between 4.0 mm and 5.0 mm by means of a first needlepunch apparatus. The needles used in the needlepunch process have a barb depth "d" of 12 µm. Thereafter, the fibrous material is conveyed to a superabsorbent application station. 40 gsm of superabsorbent (SA70 commercially available from Sumitomo Seika Chemicals Co., Ltd. Of Osaka, Japan) is applied to a top surface of the fibrous material via a gravity fed hopper. The superabsorbent is drawn into the fibrous material at a depth between 3.0 mm and 4.0 mm by means of a vacuum. Thereafter, the fibrous material 12 is conveyed to a second gravity fed hopper to apply a selected amount of a second plurality of absorbent fibers to a top surface of the fibrous material. The second plurality of absorbent fibers comprises 100% viscose rayon having a denier of 4. Rayon has a density of 1.5 g/cc thus the absorbent fibers have a fiber diameter of 19 µm. 75 gsm of the rayon fibers are applied to a top surface of the fibrous nonwoven material and impregnated within the material to a depth between 1.0 mm and 3.0 mm by means of a second needlepunch apparatus. The needles used in the second needlepunch process have a barb depth "d" of 12 µm. The final absorbent material has a thickness of 2.5 mm.

## Claims

1. A method for making an absorbent material (10) comprising the steps of:
providing a fibrous material (12) including a plurality of individual fibers (14) forming a fiber matrix (16);
depositing a plurality of absorbent fibers (18) on a top surface (30) of the fibrous material (12); and
impregnating the plurality of absorbent fibers (18) into the fiber matrix (16) by means of a needlepunch process, wherein each of the plurality of individual fibers (14) has a fiber diameter that is at least 1 µm greater than a fiber diameter of each of the absorbent fibers (18).

2. The method according to claim 1, wherein each of the plurality of individual fibers (14) has a fiber diameter within the range of between 11 µm and 100 µm.

3. The method according to claim 1 or claim 2, wherein each of the plurality of absorbent fibers (18) has a fiber diameter within the range of between 10 µm and 40 µm.

4. The method according to any one of claims 1 to 3, wherein the fibrous material (12) has a thickness prior to the plurality of absorbent fibers (18) being impregnated within the fibrous material (12) and wherein the absorbent material (10) has a thickness after the absorbent fibers (18) have been impregnated within the fibrous material (12), wherein a percent change between the thickness of the fibrous material (12) prior to the plurality of absorbent fibers (18) being impregnated therein and a thickness of the absorbent material (10) after the absorbent fibers (18) have been impregnated within the fibrous material (12) is less than 50%, or less than 30%, or less than 15%.

5. The method of any one of claims 1 to 4, wherein the fibrous material (12) is a fibrous non-woven material, wherein the fibrous non-woven material is preferably formed from a plurality of fibers selected from the group consisting of polyester, nylon, co-polyester, polyethylene, polypropylene, polylactic acid and combinations thereof

6. The method according to claim 5 wherein the fibrous non-woven is made by one of an airlaid process, a card and bind process or a resin and adhesive bond process.

7. The method of any one of claims 1 to 6, wherein the plurality of absorbent fibers (18) are selected from the group consisting of hard wood pulp, soft wood pulp, rayon, cotton, and combinations thereof.

8. The method according to any one of claims 1 to 7, wherein the needlepunch process is carried out by means a plurality of individual pins adapted to impregnate the absorbent fibers within the fiber matrix.

9. The method according to claim 8, wherein each of the plurality of pins includes a barb having a barb depth and wherein said barb depth is selected such that a fiber radius of each of the absorbent fibers is at least 0.5 µm smaller than the barb depth and the fiber radius of each of the individual fibers forming a fiber matrix is at least 0.5 µm greater than the barb depth.

## Patentansprüche

1. Verfahren zur Herstellung eines absorbierenden Materials (10), umfassend die Schritte:
Bereitstellung eines Fasermaterials (12), umfassend mehrere Einzelfasern (14), die eine Fasermatrix (16) bilden,
Abscheidung mehrerer absorbierender Fasern (18) auf einer Oberfläche (30) des Fasermaterials (12) sowie
Einimprägnierung der mehreren absorbierenden Fasern (18) in die Fasermatrix (16) durch Vernadeln, wobei die mehreren Einzelfasern (14) jeweils über einen um mindestens 1 µm größeren Faserdurchmesser als jede der absorbierenden Fasern (18) verfügen.

2. Verfahren nach Anspruch 1, bei dem die mehreren Einzelfasern (14) jeweils über einen Faserdurchmesser zwischen 11 µm und 100 µm verfügen.

3. Verfahren nach Anspruch 1 oder 2, bei dem die mehreren absorbierenden Fasern (18) jeweils über einen Faserdurchmesser zwischen 10 µm und 40 µm verfügen.

4. Verfahren nach einem der Ansprüche 1 bis 3, bei dem das Fasermaterial (12) vor der Einimprägnierung der mehreren absorbierenden Fasern (18) innerhalb des Fasermaterials (12) über eine Stärke verfügt und bei dem das absorbierende Material (10) nach der Imprägnierung der absorbierenden Fasern (18) innerhalb des Fasermaterial (12) über eine Stärke verfügt, wobei eine prozentuale Änderung zwischen der Stärke des Fasermaterials (12) vor der Einimprägnierung der mehreren absorbierenden Fasern (18) darin und einer Stärke des absorbierenden Materials (10) nach der Einimprägnierung der absorbierenden Fasern (18) innerhalb des Fasermaterials (12) weniger als 50% oder weniger als 30% oder weniger als 15% beträgt.

5. Verfahren nach einem der Ansprüche 1 bis 4, bei dem es sich bei dem Fasermaterial (12) um ein Faservlies handelt, wobei das Faservlies bevorzugt aus mehreren Fasern ausgewählt aus der Gruppe bestehend aus Polyester, Nylon, Copolyester, Polyethylen, Polypropylen, Polymilchsäure und deren Kombinationen gebildet ist.

6. Verfahren nach Anspruch 5, bei dem das Faservlies durch Luftlegung, mittels Krempeln und Bindemittel oder mittels Harz und Verklebung hergestellt ist.

7. Verfahren nach einem der Ansprüche 1 bis 6, bei dem die mehreren absorbierenden Fasern (18) ausgewählt sind aus der Gruppe bestehend aus Laubholzzellstoff, Nadelholzzellstoff, Reyon, Baumwolle und deren Kombinationen.

8. Verfahren nach einem der Ansprüche 1 bis 7, bei dem das Vernadeln mittels mehrerer Einzelstifte erfolgt, welche zur Einimprägnierung der absorbierenden Fasern innerhalb der Fasermatrix entsprechend angepasst sind.

9. Verfahren nach Anspruch 8, bei dem die mehreren Stifte jeweils einen Widerhaken mit einer Widerhakentiefe aufweisen, wobei die Widerhakentiefe so gewählt ist, dass ein Faserradius der absorbierenden Fasern jeweils um mindestens 0,5 µm kleiner als die Widerhakentiefe ist und der Faserradius der eine Fasermatrix bildenden Einzelfasern jeweils um mindestens 0,5 µm größer als die Widerhakentiefe ist.

## Revendications

1. Procédé pour la fabrication d'un matériau absorbant (10) comprenant les étapes consistant à :
fournir un matériau fibreux (12) comprenant une pluralité de fibres individuelles (14) formant une matrice de fibres (16) ;
déposer une pluralité de fibres absorbantes (18) sur une surface supérieure (30) du matériau fibreux (12) ; et
faire pénétrer la pluralité de fibres absorbantes (18) dans la matrice de fibres (16) au moyen d'un processus d'aiguilletage,
dans lequel chaque fibre individuelle de la pluralité de fibres individuelles (14) a un diamètre de fibre qui est au moins 1 µm plus grand qu'un diamètre de fibre de chacune des fibres absorbantes (18).

2. Procédé selon la revendication 1, dans lequel chaque fibre individuelle de la pluralité de fibres individuelles (14) a un diamètre de fibre dans la plage comprise entre 11 µm et 100 µm.

3. Procédé selon la revendication 1 ou la revendication 2, dans lequel chaque fibre absorbante de la pluralité de fibres absorbantes (18) a un diamètre de fibre dans la plage comprise entre 10 µm et 40 µm.

4. Procédé selon l'une quelconque des revendications 1 à 3, dans lequel le matériau fibreux (12) a une épaisseur avant que la pluralité de fibres absorbantes (18) soient amenées à pénétrer à l'intérieur du matériau fibreux (12) et dans lequel le matériau absorbant (10) a une épaisseur après que les fibres absorbantes (18) ont été amenées à pénétrer à l'intérieur du matériau fibreux (12), un pourcentage de changement entre l'épaisseur du matériau fibreux (12) avant que la pluralité de fibres absorbantes (18) y aient été amenées à pénétrer et une épaisseur du matériau absorbant (10) après que les fibres absorbantes (18) ont été amenées à pénétrer à l'intérieur du matériau fibreux (12) étant inférieur à 50 %, ou inférieur à 30 %, ou inférieur à 15 %.

5. Procédé selon l'une quelconque des revendications 1 à 4, dans lequel le matériau fibreux (12) est un matériau non tissé fibreux, le matériau non tissé fibreux étant de préférence formé à partir d'une pluralité de fibres choisies dans le groupe constitué par un polyester, un nylon, un copolyester, un polyéthylène, un polypropylène, un poly(acide lactique) et les associations de ceux-ci.

6. Procédé selon la revendication 5 dans lequel le non-tissé fibreux est formé par l'un d'un processus air-laid, d'un processus de cardage et liage ou d'un processus de collage de résine et d'adhésif.

7. Procédé selon l'une quelconque des revendications 1 à 6, dans lequel la pluralité de fibres absorbantes (18) sont choisies dans le groupe constitué par la pâte de bois de feuillus, la pâte de bois de résineux, la rayonne, le coton et les associations de ceux-ci.

8. Procédé selon l'une quelconque des revendications 1 à 7, dans lequel le processus d'aiguilletage est effectué au moyen d'une pluralité d'aiguilles individuelles conçues pour faire pénétrer les fibres absorbantes à l'intérieur de la matrice de fibres.

9. Procédé selon la revendication 8, dans lequel chaque aiguille de la pluralité d'aiguilles comprend un ardillon ayant une profondeur d'ardillon et dans lequel ladite profondeur d'ardillon est choisie de façon telle qu'un rayon de fibre de chacune des fibres absorbantes est au moins 0,5 µm plus petit que la profondeur d'ardillon et le rayon de fibre de chacune des fibres individuelles formant une matrice de fibres est au moins 0,5 µm plus grand que la profondeur d'ardillon.
